

April 29, 1930.

E. G. GILSON

1,756,857

HARD METAL COMPOSITION AND METHOD OF MAKING THE SAME

Original Filed April 28, 1927



Inventor:  
Emery G. Gilson,  
by *Wendell S. Lewis*,  
His Attorney.

## UNITED STATES PATENT OFFICE

EMERY G. GILSON, OF COLONIE, NEW YORK, ASSIGNOR TO GENERAL ELECTRIC COMPANY, A CORPORATION OF NEW YORK

**HARD-METAL COMPOSITION AND METHOD OF MAKING THE SAME**

Application filed April 28, 1927, Serial No. 187,328. Renewed June 11, 1929.

The present invention relates to a hard metal composition and more particularly to a method of forming such a composition into a hard, dense mass which is suitable for use as 5 a machine cutting tool, wire drawing die or the like.

Metallic compositions, consisting largely of a refractory metal of the sixth group of the periodic table, have heretofore been made 10 by mixing, for example, as disclosed in the patent to Schröter No. 1,549,615, powdered tungsten carbide and a powdered auxiliary metal, such as cobalt, forming the powdered mixture in a mold under pressure, and then 15 heating the molded bar to its sintering temperature. Metallic compositions formed in this manner may contain from about 5 to about 20 per cent of auxiliary metal, and the finished product is suitable for use as dies, 20 cutting tools, or the like depending on the amount of auxiliary metal employed. The above process, it will be noted, involves four separate and distinct steps, viz., forming tungsten carbide, mixing the latter with an 25 auxiliary metal, pressing the mixture, and sintering. The process of forming the carbide particularly involves difficulties since it necessitates the employment of high temperatures and requires three hours or more for 30 its completion.

In the copending application of Samuel L. Hoyt, Serial No. 181,536, filed April 6, 1927, entitled "Hard metal compositions and methods of making the same," there is disclosed a 35 further method for forming a hard, tough, metallic structure, the latter method comprising mixing a carbide such as tungsten carbide with an auxiliary metal such as cobalt and simultaneously applying heat and pressure to the mixture.

It is one of the objects of the present invention to provide a more simple and inexpensive process than that heretofore employed for making metal compositions of the 45 above character. This object has been accomplished by omitting the step in the former processes which involves the preformation of tungsten carbide and by performing the necessary steps involved in forming the metal com-

position into a hard, dense mass in a single operation.

In carrying out the invention a metal of the sixth group of the periodic table, preferably tungsten in powdered form, is mixed 55 with powdered carbon and a powdered auxiliary or binder metal of the iron group, preferably cobalt. The elements are thoroughly mixed and then subjected to pressure in a reducing atmosphere for a short time, approximately five minutes, at the sintering temperature of the mixture. The close contact of the particles, due to the pressure employed, assists in shortening the time necessary for the formation of tungsten carbide at this temperature. The rapidity of formation of the carbide moreover is materially facilitated by the presence of cobalt or other metal of the iron group. The product obtained by such a process is very hard and strong, substantially 60 free from porosity, and particularly desirable 65 for use as machine cutting tools and dies.

The novel features which I believe to be characteristic of my invention are set forth with particularity in the appended claims. 70 My invention itself, however, will best be understood from reference to the following specification taken in connection with the accompanying drawing in which the single figure shows diagrammatically a perspective 75 view partly in section and partly in elevation of a mold and assembled electrodes whereby my invention may be carried into effect.

The elements, preferably finely divided tungsten, carbon and cobalt, which comprises 80 the finished product, are thoroughly mixed in any suitable manner and placed in a carbon mold 1 which may have a rectangular or other suitable opening 2 extending therethrough. An electrode 3 fits slidably in the lower part 85 of opening 2 and receives the powdered mixture thereon. A second electrode 4 is slidably mounted in the upper part of the opening. Current is supplied to the electrodes 3 and 4 through metallic connectors 5 and 6, while 90 pressure is simultaneously applied through the electrodes to the powdered materials 7. A pressure of approximately 1,000 pounds per square inch is applied to the powdered material at temperatures varying from 1300 to 100

1450° C. depending on the mixture employed. The temperature employed will be the sintering temperature of the mixture and should be maintained from one to several minutes to obtain the best results.

5 The amounts of powdered or finely divided materials employed may be varied if desired. The carbon content, however, should not be less than three nor more than ten per cent of the tungsten content. A mixture containing an amount of carbon equal approximately to 6 per cent of the tungsten content will be found to give very satisfactory results. The amount of auxiliary metal contained in the 10 mixture may be about 5 per cent or more of the total content of the composition. Good cutting tools and dies have been obtained by employing either 5 per cent or 25 per cent of auxiliary metal.

0 While I have found that the elements, tungsten, cobalt and carbon, provide the most satisfactory composition for use as cutting tools and dies other elements of the sixth group of the periodic table may be substituted for the 5 tungsten and likewise other metals of the iron group may be substituted for the cobalt if desired.

What I claim as new and desire to secure by Letters Patent of the United States is:

10 1. The method of producing a metallic structure consisting largely of tungsten but containing appreciable amounts of carbon and an element of the iron group, which comprises mixing powdered tungsten, carbon and an element of the iron group, and applying pressure thereto at the sintering temperature of the mixture.

15 2. The method of making metallic structure suitable for use as a cutting tool, which comprises applying pressure to a finely divided mass of tungsten, carbon and cobalt at approximately the sintering temperature of the mass.

3. The method of making a cutting tool, 5 which comprises mixing in finely divided form an element of the sixth group of the periodic table, an element of the iron group and carbon, and applying pressure thereto at the sintering temperature of the mixture.

0 4. A metal cutting tool formed by the simultaneous application of heat and pressure to powdered tungsten, carbon and cobalt.

5 5. The method of forming a metallic structure consisting largely of tungsten but containing appreciable amounts of carbon and cobalt, which comprises mixing powdered tungsten, carbon and cobalt in the desired proportions, heating the powdered materials to the sintering temperature of the mixture, and applying pressure thereto.

6. The method of forming a metallic structure consisting largely of tungsten but containing appreciable amounts of carbon and cobalt, which comprises mixing powdered tungsten, carbon and cobalt in the desired

proportions, heating the powdered materials to the sintering temperature of the mixture, and simultaneously applying pressure thereto.

7. The method of forming a metallic structure consisting largely of tungsten but containing from 5 to 25% cobalt and about 5.4% to 4.2% carbon, which comprises mixing powdered tungsten, carbon and cobalt in the above proportions, heating to the sintering temperature of the mixture and applying pressure thereto. 75

8. The method of forming a metallic structure consisting largely of tungsten but containing from 5 to 25% cobalt and about 5.4% to 4.2% carbon, which comprises mixing powdered tungsten, carbon and cobalt in the above proportions, heating to the sintering temperature of the mixture and simultaneously applying pressure thereto. 80

9. The method of forming a metallic structure consisting of tungsten carbide and an appreciable amount but not more than 25% of cobalt which comprises mixing the elements, tungsten, carbon and cobalt in powdered form, heating them to the sintering temperature of the mixture and applying pressure thereto. 85

10. The method of forming a metallic structure consisting of tungsten carbide and an appreciable amount but not more than 25% of cobalt which comprises mixing the elements, tungsten, carbon and cobalt in powdered form, heating them to the sintering temperature of the mixture and simultaneously applying pressure thereto. 90

11. The method of making a hard strong metal composition consisting mainly of a metal of the 6th group of Mendelejeff's periodic table but containing appreciable amounts of carbon and metal of the iron group, which comprises mixing said metal of the 6th group and said carbon, while uncombined with respect to one another, with said metal of the iron group, and consolidating 105 said mixture into a hard strong body.

12. The method of making a hard strong metal composition consisting mainly of tungsten but containing appreciable amounts of carbon and cobalt, which comprises mixing free carbon with tungsten and cobalt, and consolidating the mixture into a hard strong body. 115

13. The method of making a hard strong metal composition consisting mainly of tungsten carbide but containing an appreciable amount of cobalt, which comprises providing a mixture containing free carbon, tungsten and cobalt, and consolidating the mixture into a hard strong body. 120

14. The method of making a hard strong metal composition consisting mainly of tungsten but containing appreciable amounts of carbon and cobalt, which comprises mixing the tungsten, carbon and cobalt each in 130

powdered form, and while uncombined with one another, and consolidating the mixture into a hard strong body by the application of heat and pressure thereto.

5 15. The method of making a hard strong metal composition consisting substantially of tungsten, carbon and cobalt, the cobalt forming an appreciable amount but not more than 25% of the composition, which comprises 10 mixing free carbon with tungsten and cobalt, and consolidating the mixture into a hard strong body by the application of heat and pressure thereto.

15 16. The method of making a carbide of an element of the 6th group of Mendelejeff's periodic table, which comprises mixing free carbon with said element and metal of the iron group and heating the mixture to an elevated temperature.

20 17. The method of making tungsten carbide, which comprises providing a mixture containing tungsten, cobalt and free carbon, and heating the mixture.

25 18. The method of accelerating the formation of tungsten carbide, which comprises heating a finely divided mixture consisting mainly of tungsten but containing appreciable amounts of cobalt and free carbon.

In witness whereof, I have hereunto set  
30 my hand this 27th day of April, 1927.

EMERY G. GILSON.

35

40

45

50

55

60

65